

1,237,551.

W. A. PHILLIPS,  
PROCESS OF DRYING EXPLOSIVES.  
APPLICATION FILED AUG. 13, 1913.

Patented Aug. 21, 1917.  
2 SHEETS—SHEET 1.

Fig. 1



Fig. 2



Witnesses:

A. C. Seagren  
Matelle J. Ware

William A. Phillips, Inventor

By his Attorneys  
Brindleybright

1,237,551.

W. A. PHILLIPS.  
PROCESS OF DRYING EXPLOSIVES.  
APPLICATION FILED AUG. 13, 1913.

Patented Aug. 21, 1917.

2 SHEETS—SHEET 2.



Witnesses:

*D. C. Seagren*  
Matelle J. Ware

*William A. Phillips* Inventor  
By his Attorneys  
Pindler & Wright

# UNITED STATES PATENT OFFICE.

WILLIAM A. PHILLIPS, OF PHILADELPHIA, PENNSYLVANIA, ASSIGNOR TO E. I. DU PONT DE NEMOURS POWDER COMPANY, OF WILMINGTON, DELAWARE, A CORPORATION OF NEW JERSEY.

## PROCESS OF DRYING EXPLOSIVES.

1,237,551.

Specification of Letters Patent. Patented Aug. 21, 1917.

Application filed August 13, 1913. Serial No. 784,486.

To all whom it may concern:

Be it known that I, WILLIAM A. PHILLIPS, of Philadelphia, in the county of Philadelphia and in the State of Pennsylvania, have invented a certain new and useful Improvement in Processes of Drying Explosives, and do hereby declare that the following is a full, clear, and exact description thereof.

- 10 My invention relates to a process of drying explosives of many different kinds and the product obtained thereby, but it has special reference to drying smokeless powder. It is to be understood, however, that my invention is applicable to the drying of many different products of similar kind which are of such a nature that they may be dried in accordance with my invention hereinafter set forth.
- 15 Hitherto, it has been customary to recover the solvents used in producing smokeless powders, by methods which have been disadvantageous in many ways. Smokeless powders have been previously dried by the circulation of hot air through the powder grains. The hot air thus circulated through the powder grains carried off the greater part of the solvent, this air being subsequently conducted to a condenser to remove 20 the solvents from the current of air; the maximum amount of solvent that could be recovered in this manner was about sixty per cent.; and it was necessary to treat the powder for a further period of from one 25 to four months in order to reduce the solvent still contained in the powder to a sufficient extent to give proper ballistic results. But even after the drying of the powder for this extended period, a comparatively large 30 percentage of solvent was still left in the powder, which solvent was not entirely uniformly distributed in the grains thereof, and the grains furthermore showed signs of strain and distortion. Again, the solvent 35 retained in the grains is liable to become partially oxidized, to form hydrogen peroxid, ozone, acids, and other objectionable substances which may decompose the powder. And the vapors of solvents evolved 40 from the powder during storage in airtight containers are capable of forming an explosive mixture with the air, resulting at

times in an explosion. Furthermore, the very long heating necessary to recover the solvent and in the dry-house shortens the 55 life of the powder by quickening the spontaneous decomposition of the nitric esters, thus leading to the possibility of grave accidents. A further disadvantage of said heating is the fact that a portion of the 60 stabilizers is caused to escape by volatilization. A further frequent cause of decomposition is the presence of bacteria in the powder.

The object of my invention is to provide 65 a process and product whereby the above disadvantages are avoided. By means of my invention, furthermore, a more complete recovery of the solvents is obtained, and the powders thus produced show remarkable 70 results in ballistic qualities, keeping qualities, resistance to the injurious influence of moisture, heat, etc.

My invention comprises in general the 75 drying of powder by the use of a liquid, such for example, as oil instead of by the application of air. The oil used for this purpose should preferably be stable and not subject to chemical change. It must be free from acid, have a high flash point, and possess a low viscosity and a low solidifying 80 point. An oil of this character will penetrate the pores of the powder grains and will extract the solvents and absorb the same 85 therefrom by osmosis. The even drying avoids the strain and distortions which were produced in the grains dried by former processes.

My invention is capable of being carried 90 out in many different ways, but, for the purpose of illustration, I have shown certain apparatus which may be used for the purpose of carrying out my invention, in the accompanying drawings, in which,

Figure 1 is a diagrammatic representation 95 of one form of apparatus that may be used for carrying out my invention,

Fig. 2 is a diagrammatic representation 100 of another form of apparatus which may be used for carrying out my invention.

Figs. 3 and 4 are diagrammatic representations of details of an apparatus of the type shown in Fig. 2,

Fig. 5 is a diagrammatic representation

of another arrangement of apparatus which may be used for carrying out my invention, and

5 Figs. 6 and 7 are diagrammatic representations of details of a type of apparatus such as that shown in Fig. 5.

Reference being had particularly to Fig. 1, the powder from the cutters is conducted through a funnel 1, the lower end of which 10 is sealed within a body of oil 2 contained within a tank 3. At its lower end the tank 3 has baffles 4 to guide the grains of powder to a screw conveyer 5 located in the bottom of the tank 3 and having a shaft 6 and 15 operating handle 7 which extends laterally out through a horizontal extension 8 attached to the lower end of the tank 3. When the powder grains have thus been received by the tank 3 they are thereafter 20 conveyed by the conveyer 5 to a vertical drying chamber 9 which is attached to the end of the horizontal extension 8. The lower end of the vertical drying chamber is closed by a cover 10. When the powder has been treated 25 in the drying chamber 9 the conveyer 5 is moved to the left of the apparatus, as shown in Fig. 1, and a valve 11, located in the horizontal section 8, is moved upwardly so as to separate the tank 3 from the drying 30 chamber 9. Any vapors of solvents, such, for example, as ether, alcohol, acetone, etc., that are produced in the tank 3 are conducted upwardly through a pipe 12 to a condenser 13, from which the liquid solvents 35 are conducted to a receptacle 14. The condenser 13, as in the case of all the other condensers to be referred to in this application, may be cooled by a current of water, or in any other desired manner. The solvent 40 vapors which are formed in the drying chamber 9 are conveyed through a pipe 15 to a condenser 16, from which the condensed solvents are collected by means of a receptacle 17. Means are provided for circulating 45 a body of oil in the tank 3 and in the drying chamber 9 and also for withdrawing the oil from the drying chamber 9. This is accomplished by means of an oil chamber 18 having a heating coil 19 therein preferably 50 provided with a supply of steam. The heating chamber 18 is connected to the top of the tank 3 by a valved pipe 20 and to the bottom of the tank 3 by a valved pipe 21, the latter being provided with a circulating 55 pump 22. The oil chamber 18 is also connected to the top of the drying chamber 9 by a valved pipe 23 and to the bottom thereof by pipes 24 and 25. The pipes 24 and 25 are connected to each other by two 60 parallel pipe connections 26 and 27, each of which has a pair of valves 28, 29, 30 and 31. A pump 32 is provided in another pipe 33 which is bridged between the pipe connections 26 and 27 at points located between 65 the pairs of valves, as indicated in Fig. 1.

Any vapors that are formed in the oil chamber 18 are conveyed upwardly through a pipe 34 to a condenser 35, from which the condensed solvents are collected by means of a receptacle 36.

I have shown somewhat similar arrangements in the other figures. In the arrangement shown in Figs. 2, 3 and 4, the powder grains are delivered into a series of movable containers or drying chambers 37, each of 70 which has a column 38, which may be connected to a pipe 39 leading to a condenser 40, having a discharge receptacle 41 for the condensed solvents. If desired, the movable containers 37 may have doors 37<sup>a</sup> near the 80 bottom thereof to facilitate the removal of the powder. The same condenser 40 is arranged in this instance to receive vapors by means of a pipe 42 from an oil chamber 43, provided with heating coils 44 in the same 85 manner as in the arrangement shown in Fig. 1. Pipes similar to those shown in Fig. 1 as being connected to the oil chamber 18 are provided in this instance. Circulating pipes 45 and 46 are provided to circulate 90 heated oil through the containers 37 and a third pipe 47 is provided to draw the oil from the containers. Pipes 46 and 47 are supplied with pumps 48 and 49 to bring about the movement of the oil in the pipes 95 46 and 47. As shown in Fig. 4, each of the containers may be carried upon a skid 50 having wheels 51 so as to permit the same to be readily moved from one point to another in the plant.

The arrangement shown in Figs. 5, 6 and 7 is constructed in a manner somewhat similar to that shown in Figs. 2, 3 and 4. In this instance, however, the powder grains are carried in a wire cage or bag 52 made in 105 any desired manner, said wire cage or bag 52 being received in movable containers or drying chambers 53 situated upon movable skids 54 having wheels 55. The top of each of the movable containers 53 has a water 110 seal 56 in which is received the larger end of a solvent header 57. The smaller ends of the solvent headers 57 communicate with a common pipe 58 leading to a condenser 59 having a discharge receptacle 60. In this 115 instance, an oil tank 61 is provided, having pipes 62 and 63 connected by means of branches 64 and 65 with the containers 53 in order to circulate oil through the same. In this modification a pair of valves 66 and 120 67 are provided in the pipe 62 and a similar pair of valves 68 and 69 are provided in the pipe 63. A pump 70 is located in a pipe 71 bridging the two pipes 62 and 63 between the two pairs of valves just referred to. At their 125 ends the pipes 62 and 63 may be connected together and have a valve 72 at the point where the pipes are connected. In this arrangement the oil is not heated in the oil chamber 61, but there may be provided in- 130

stead heating coils 73 in each of the chambers 53, said heating coils being connected by means of valved pipes 74 and 75 to steam pipes 76 and 77 in order to provide a supply 5 of steam for the heating coils.

In the operation of my process, I shall refer to the same first in connection with the use of the apparatus shown in Fig. 1. The powder from the cutters is conveyed into the 10 tank 3 filled with a suitable body of oil to effect the drying of the powder. The powder is conveyed into the tank 3 through the funnel 1, the lower end of which is sealed in the body of oil, so that no vapors arising 15 from the powder and the oil can escape from the tank 3. As soon as the powder has become immersed in the oil, the transfer of the solvent from the powder to the oil begins even at ordinary temperatures, and the volume 20 of the liquid increases as the volume of the powder decreases. The transfer of solvent from the powder to the oil may be hastened by circulating warm or hot oil from the oil chamber 18, the oil in which may be 25 heated by means of the steam coils 19 therein. In order to effect the circulation of the oil at this period in the process, the pump 22 may be operated so as to circulate the oil from the oil chamber 18 through the valved 30 pipes 20 and 21. Any solvent vapors which arise from the tank 3 during such treatment are condensed in the condenser 13 and conveyed to receptacle 14. The powder which has been subjected to this preliminary treatment 35 may be then removed by means of the conveyer 5 to the drying chamber 9. If desired, the process may, in fact, be carried out continuously by continually feeding in the powder through the funnel 1 and intermittently removing the same through the door 40 10 from the drying chamber 9, in the manner to be hereinafter described. If desired, after the powder grains have been conveyed to the drying chamber 9, the conveyer 5 may 45 be withdrawn to the left of valve 11 shown in Fig. 1 and said valve 11 may be closed so as to separate the tank 3 from the drying chamber 9. Oil may then be circulated, if desired, in the drying chamber 9 by means of 50 the pump 32, the valves 28, 29, 30 and 31 being in proper position, until the solvent in the powder has been removed. Any vapors which are evolved by the treatment in the 55 drying chamber 9 are condensed in the condenser 16 and recovered in the receptacle 17, and any vapors which are evolved at any stage in the process from the oil chamber 18 are condensed in the condenser 35 and collected in the receptacle 36. If now it is desired 60 to remove the powder from the drying chamber 9, the oil is withdrawn from the same by closing the valve in the pipe 23 and operating the pump 32 with the valves 28, 29, 30 and 31 in proper position for this purpose. The oil having been drained from the

drying chamber 9 in this manner, the door 10 is detached and the body of powder removed from the drying chamber. If desired, the powder removed from the drying chamber 9 can be subjected to a washing operation with gasolene, or other solvent of the oil remaining upon the powder, so as to remove said oil therefrom. And to remove the gasolene or other similar solvent the powder may be subjected to aeration. 70

The operation of the form of apparatus shown in Figs. 2, 3 and 4 is, in general, the same as in the case of the operation of my invention with the apparatus shown in Fig. 1. It differs, however, in the following respects: The movable containers 37, having been charged with a quantity of powder while on the movable skids, said containers are moved into a position in which the several pipes of the apparatus may be connected, and the solvent pipes 38 are then connected to the pipe 39, and pipes 45, 46 and 47 are also connected to the containers 37. Heated oil may now be circulated from the oil chamber 43 to the several containers 37 until the powder therein has been sufficiently dried. Meanwhile, any vapors evolved from the containers 37 and the oil chamber 43 are condensed in the condenser 40 and recovered in receptacle 41. After 80 the powder has been dried in this manner, the oil circulating pipes are closed by turning the valves located therein and the oil in the containers 37 is removed by means of pipe 47 through the operation of the pump 49. The containers 37 may now be disconnected and conveyed to any suitable place where the powder located therein may be subjected to a washing operation with gasolene, or other suitable solvent of the oil, 85 so as to remove the remainder of the oil present on the powder. The solvent remaining on the powder may be removed by aeration, if desired. In order to economize space, the several containers may be operated when nearly filled with powder. It is to be understood, however, that the several containers 37 may be operated in such a manner that the treatment of the bodies of powder in the several containers may be 90 finished in sequence so as to economize time, labor, etc. It is also to be understood that, if desired, the circulation of the oil may be effected through the several containers in sequence on the counter current principle, 95 100 so that the body of powder which has been subjected to the longest period of treatment is being subjected to oil coming direct from the oil chamber, while the other containers receive the oil from the first mentioned container in sequence. 110

The process as carried out in the form of apparatus shown in Figs. 5, 6 and 7 is substantially the same as that carried out in the apparatus shown in Figs. 2, 3 and 4, 115 120 125 130

except in the following respects: In this instance, the cages 52, having been charged with suitable quantities of powder, are placed in the receptacles 53 and are then 5 moved upon the movable skids 54 to their proper positions to permit the various pipes of the drying system to be connected thereto. The solvent headers 57 are then placed in position so that they are connected to the 10 common pipe 58, and the remaining pipes of the system are connected to the containers 53. Oil is now circulated from the oil receptacle 61 through the containers 53 and, if it is desired to circulate a heated current 15 of oil, currents of steam are led through the heating coils 73 in the bottom of the containers. Any vapors produced in the system in this instance are evolved from the containers 53 and are thereupon condensed 20 in the condenser 59 and recovered from the receptacle 60. When the drying operation has been completed, the oil present in the containers is removed by means of the pump 70 and conveyed into the oil chamber 61. 25 In this instance, the several containers may be operated in serial order in the manner described in connection with the apparatus shown in Figs. 2 to 4.

In the treatment by means of oil in the 30 process as carried out in connection with the apparatus shown in the several modified forms already described, the oil is caused to mix homogeneously, so that all portions of the oil are brought into intimate and uniform contact with the powder under treatment. As a result, there is also an agitation within the bodies of powder which carries off any air bubbles. Furthermore, the circulation of the liquid through the bodies 35 of powder distributes the heat uniformly throughout the same, so that thereby the solvent is uniformly transferred to the oil in an efficient manner. Powder which is treated in this manner may be dried in a 40 few days, whereas the previous method in use, involving the application of heated air, required a period of several months to complete the drying operation. The use of oil causes the powder to be more quickly dried, 45 owing to the greater conductivity of oil for heat and, furthermore, permits the transfer of a large number of thermal units to the powder in a short time without unduly raising the temperature thereof. Furthermore, 50 there is a more complete contact between the oil and the powder, as the oil penetrates and permeates the grains thoroughly. The operation is such as to cause an efficient removal of the solvent from the powder by 55 osmosis. The treatment of powder in accordance with my invention is for such a short period of time that practically no deterioration of the powder takes place, and there is consequently avoided the disadvantageous result of previous processes in which 60

the rate of spontaneous decomposition increases rapidly during storage, the rapidity of decomposition being greater the longer the powder has been subjected to elevated temperatures. It will thus be seen that powders dried in accordance with my invention have a longer period of life and may be carried in storage and handled with much greater safety than the powders dried by former processes. Furthermore, on account 70 of the absence of solvent vapors evolved during storage, there is not the tendency to form explosive mixtures with air, which makes powders dried by previous processes unsafe when stored for a considerable length 75 of time. The circulation of the oil, in addition to expelling air bubbles, also has the effect of expelling the water which is found in the powder mass and which has been left therein from the solvents used, which solvents contain about 7% of water, and also expelling the microscopic drops of water which have condensed on the grains during 80 their shaping and cutting. The presence of such moisture would contribute considerably 85 to the deterioration of the powder, a fact which is proven by the short life of powders in moist climates. Besides being anhydrous, the powders dried in accordance 90 with my invention are non-hygroscopic, owing to the fact that a slight amount of the oil remains in the grains after the treatment. Another advantage of my invention is that it does not result in the volatilization 95 of stabilizing agents, such, for example, as diphenylamin, which are incorporated in powders to neutralize the traces of acid fumes evolved during spontaneous decomposition. If desired in the treatment in accordance 100 with my process, in order to avoid any loss of the diphenylamin or other stabilizers by solution in the oil, a quantity of the stabilizer may be added to the oil before treatment of the powder. The temperature 105 of the oil in the treatment of the powder may be as high as 100° C., or even higher, and the various parts of the apparatus may be constructed, if desired, in such a manner as to make use of such temperatures. It will 110 also be seen that the treatment in accordance 115 with my invention destroys all bacteria contained in the powder by sterilization.

In addition to the advantages pointed out above, there are still further advantages in the use of my invention. The solvents, such 120 as ether, alcohol, acetone, etc., are almost completely recovered. Furthermore, it is found that powder treated in the manner indicated retains its ballistic properties constant. If desired, the powder may be dried 125 without any elevation of temperature above atmospheric temperature. The powder treated in the manner indicated, in accordance with my invention, is comprised of grains that are homogeneous in structure and 130

show neither distortion nor strain. There is an entire absence of danger due to super-heating, formation of electric charges, sparks, etc., during the treatment. By using 5 a circulating current of oil, the drying operation may be more readily controlled than in the case of previous processes. Again, the circulating oil does not depend, as in the case of heated air, for the removal of 10 solvent through the action of vapor tension, but is accomplished by osmosis. The amount of heat expended in the process is very small and the plant necessary for carrying out the process is not large.

15 While I have described my invention in detail, I wish it to be understood that many changes may be made therein without departing from the spirit of my invention.

I claim:

20 1. The process which comprises removing a liquid from a solid material soluble therein, by bringing said material into contact with a non-solvent oil miscible with said liquid.

25 2. The process which comprises removing a liquid from a smokeless powder soluble therein, by bringing said material into contact with a non-solvent oil miscible with said liquid.

30 3. The process which comprises removing a liquid from a smokeless powder soluble therein, by bringing said material into contact with a non-solvent oil miscible with said liquid, by circulating a body of the heated 35 oil through a body of the powder.

40 4. The process which comprises removing a liquid from a smokeless powder soluble therein, by bringing said material into contact with a non-solvent oil miscible with said liquid, by circulating a body of the heated oil through a body of the powder, and drawing off the oil.

45 5. The process which comprises removing a liquid from a smokeless powder soluble therein, by bringing said material into contact with a non-solvent oil miscible with said liquid, by circulating a body of the heated oil through a body of the powder, drawing off the oil, and removing the remainder of 50 the oil by washing with a solvent thereof.

55 6. The process which comprises removing a liquid from a smokeless powder soluble therein, by bringing said material into contact with a non-solvent oil miscible with

said liquid, by circulating a body of the heated oil through a body of the powder while recovering any escaping solvent vapors, and drawing off the oil.

7. The process which comprises removing a liquid from a smokeless powder soluble 60 therein, by bringing said material into contact with a non-solvent oil miscible with said liquid, by circulating a body of the heated oil through a body of the powder while recovering any escaping solvent 65 vapors, drawing off the oil, and removing the remainder of the oil by washing with a solvent thereof.

8. The process which comprises removing a nitrocellulose solvent and water from 70 smokeless powder by applying oil thereto.

9. The process which comprises drying smokeless powder by subjecting the same to a body of an oil containing a stabilizing 75 agent.

10. The process which comprises drying smokeless powder by subjecting the same to a body of a heated oil containing diphenylamin.

11. The process which comprises removing a nitrocellulose solvent and air-bubbles 80 from smokeless powder by applying oil thereto.

12. The continuous process which comprises feeding a quantity of smokeless powder 85 containing a solvent into a body of heated oil, circulating the body of oil in the body of powder, recovering solvent vapors escaping from the body of oil, segregating the treated powder in the body of oil, cutting off the segregated body of powder 90 from the main body of oil, withdrawing the oil from the segregated powder, washing the same with a solvent of the oil, removing the solvent by aeration, and feeding 95 into the main body of oil another body of powder containing a solvent to be treated.

13. The process which comprises removing solvent from smokeless powder by osmosis through the application of an oil 100 to the smokeless powder miscible with said solvent.

In testimony that I claim the foregoing I have hereunto set my hand.

WILLIAM A. PHILLIPS.

Witnesses:

S. W. FOULKROD,  
E. N. KEMP.